

# United States Patent Office

3,161,503

Patented Dec. 15, 1964

1

3,161,503

## CORROSION RESISTANT ALLOY

Gilbert A. Lenning, Las Vegas, and Harry W. Rosenberg, Henderson, Nev., assignors to Titanium Metals Corporation of America, New York, N.Y., a corporation of Delaware

No Drawing. Filed Sept. 27, 1961, Ser. No. 141,903

2 Claims. (Cl. 75—174)

This invention relates to corrosion resistant alloys and more particularly to alloys containing titanium and tantalum having corrosion properties approaching those of pure tantalum, and also being thermally stable.

The excellent corrosion resistant properties of alloys containing titanium and relatively large percentage of tantalum are known. Such alloys are described in U.S. Patent 2,964,399. In addition to binary alloys of titanium and tantalum, alloys in which the tantalum is in part replaced by columbium are also described in this patent. Such alloys are substantially less costly than pure tantalum but approach the corrosion resistance of tantalum in their ability to withstand corrosive effects of solutions such as boiling hydrochloric, sulfuric, phosphoric or oxalic acids. While these alloys do possess remarkable and valuable corrosion resistant properties, it has been found that they are not thermally stable. When exposed to temperatures of the order of several hundred degrees Fahrenheit they tend to become brittle. This embrittlement can lead to catastrophic disintegration, and complete loss of their structural integrity. It is interesting to note in this connection that the reactions responsible for this embrittlement appear to be functions of both temperature and time, and while they are clearly evident after exposure of such an alloy to a temperature of several hundred degrees Fahrenheit in a relatively short space of time, the same embrittling effect occurs at lower temperatures after an extended period of time. Since, by their nature, corrosion resistant alloys are expected to provide often many years of service, even a slightly elevated temperature during their normal useful life can produce undesirable embrittlement during such a long exposure time.

2

Therefore such alloys while being extremely useful at normal or so-called room temperature are restricted in practical applications, and do not appear to be suitably employed exposed to relatively high temperatures for even a short period of time, or even moderately elevated temperatures during a long period.

It is therefore a principal object of this invention to provide an improved corrosion resistant alloy. Another object of this invention is to provide a thermally stable corrosion resistant alloy. Another object of this invention is to provide an improved thermally stable and corrosion resistant alloy having corrosion resistant properties approaching those of pure tantalum but which can be produced at substantially lower cost. Another object of this invention is to provide a corrosion resistant alloy possessing high strength together with good ductility, and which is corrosion resistant and thermally stable. These and other objects of this invention will be apparent from the following description thereof.

This invention in its broad aspects contemplates corrosion resistant alloys characterized by thermal stability, and consisting essentially of from 40 to 70% by weight tantalum, and a beta stabilizer selected from the group consisting of vanadium, molybdenum, chromium, iron and manganese and mixtures thereof in amount from 2% to 20% by weight, balance titanium. The thermal stability of the alloys of this invention is indicated by substantial retention of ductility after exposure to temperatures up to about 800° F. Optionally the alloys of this invention may include up to 2.5% by weight of aluminum, and additional advantages will be derived from its inclusion. A preferred range of beta stabilizing content is from 5% to 10% by weight within which the optimum advantages provided by the beta stabilizer inclusion are obtained. Up to 15% by weight of columbium may be employed in the alloy of this invention to replace a similar percentage of tantalum, the tantalum and columbium being present in the aggregate within the range from 40% to 70% by weight and with tantalum content 35% to 70% by weight. A particularly effective and desirable alloy composition consists essentially of about 50% by

Table I

CORROSION TESTS OF VARIOUS ANNEALED TITANIUM-TANTALUM ALLOYS IN VARIOUS BOILING MEDIA

| Heat No. | Composition      | Exposure Time, Hours | Corrosion Rate, Mils Per Year |                                    |                                    |                |
|----------|------------------|----------------------|-------------------------------|------------------------------------|------------------------------------|----------------|
|          |                  |                      | 20% HCl                       | 60% H <sub>2</sub> SO <sub>4</sub> | 80% H <sub>3</sub> PO <sub>4</sub> | 3% Oxalic Acid |
| 9151     | Ti-50Ta          | 24                   | 3.60                          | 4.07                               | —                                  | 38.5           |
| 9151     | Ti-50Ta          | 51                   | 1.81                          | 2.14                               | —                                  | 51.0           |
| 9151     | Ti-50Ta          | 168                  | 0.80                          | 0.96                               | —                                  | 47.5           |
| 9151     | Ti-50Ta          | 336                  | 0.43                          | 0.58                               | —                                  | 31.1           |
| 9151     | Ti-50Ta          | 672                  | 0.24                          | 0.47                               | —                                  | 25.3           |
| 9152     | Ti-40Ta-10Cb     | 24                   | 2.28                          | 7.39                               | —                                  | 36.1           |
| 9152     | Ti-40Ta-10Cb     | 51                   | 1.12                          | 3.74                               | —                                  | 30.5           |
| 9152     | Ti-40Ta-10Cb     | 168                  | 0.69                          | 2.46                               | —                                  | 20.2           |
| 9152     | Ti-40Ta-10Cb     | 336                  | 0.40                          | 1.75                               | —                                  | 13.8           |
| 9152     | Ti-40Ta-10Cb     | 672                  | 0.22                          | 1.71                               | —                                  | 13.9           |
| T-121    | Ti-74Ta          | 48                   | 0.1                           | —                                  | —                                  | —              |
| T-284    | Ti-70Ta          | 48                   | 0.6                           | —                                  | —                                  | —              |
| T-120    | Ti-65Ta          | 48                   | 0.3                           | —                                  | —                                  | —              |
| T-119    | Ti-62Ta          | 48                   | 0.7                           | —                                  | —                                  | —              |
| 9458     | Ti-40Ta-10Cb-2V  | 168                  | 4.8                           | 3.4                                | 3.3                                | 26.6           |
| 9459     | Ti-40Ta-10Cb-5V  | 168                  | 4.7                           | 1.9                                | 3.4                                | 20.6           |
| T-78     | Ti-40Ta-10Cb-7V  | 48                   | 8.1                           | —                                  | —                                  | —              |
| 9460     | Ti-40Ta-10Cb-10V | 24                   | 0.95                          | 9.48                               | —                                  | 50.7           |
| 9460     | Ti-40Ta-10Cb-10V | 51                   | 0.89                          | 4.88                               | —                                  | 24.2           |
| 9460     | Ti-40Ta-10Cb-10V | 168                  | 0.45                          | 2.92                               | 5.0                                | 16.5           |
| 9460     | Ti-40Ta-10Cb-10V | 336                  | 0.34                          | 1.83                               | —                                  | 10.8           |
| 9460     | Ti-40Ta-10Cb-10V | 672                  | 0.20                          | 1.81                               | —                                  | 8.3            |
| T-79     | Ti-40Ta-10Cb-12V | 48                   | 9.5                           | —                                  | —                                  | —              |
| T-80     | Ti-40Ta-10Cb-16V | 48                   | 4.9                           | —                                  | —                                  | —              |
| T-81     | Ti-40Ta-10Cb-20V | 48                   | 6.2                           | —                                  | —                                  | —              |
| 9461     | Ti-40Ta-10Cb-3Cr | 24                   | 2.62                          | 7.38                               | —                                  | 40.5           |
| 9461     | Ti-40Ta-10Cb-3Cr | 51                   | 1.21                          | 3.63                               | —                                  | 30.2           |
| 9461     | Ti-40Ta-10Cb-3Cr | 168                  | 0.75                          | 2.98                               | 3.6                                | 16.4           |
| 9461     | Ti-40Ta-10Cb-3Cr | 336                  | 0.41                          | 1.88                               | —                                  | 10.0           |
| 9461     | Ti-40Ta-10Cb-3Cr | 672                  | 0.25                          | 1.88                               | —                                  | 7.61           |

weight of tantalum, about 1.5% by weight aluminum, about 8.5% by weight vanadium, and the balance titanium. Another very desirable specific alloy composition in which a portion of the tantalum content is replaced by columbium, consists essentially of about 40% by weight tantalum, about 10% by weight columbium, about 1.5% by weight aluminum, about 8.5% by weight vanadium, and the balance titanium.

Table 1, preceding, shows the results of corrosion tests on a number of alloys whose composition is shown as percentages by weight of alloying ingredients, balance titanium. The ingredients for each alloy were melted in an arc furnace into a small ingot which was remelted several times to insure homogeneity. The remelted ingot was rolled to form sheet of thickness about 0.040 inch, and the rolled sheet was annealed at 1400°-1500° F. for a period of 1/2 to 1 hour. Sections of sheet were cut to form coupons which were immersed in boiling acids of composition shown. Corrosion rates were calculated from weight loss.

Another group of alloys were similarly fabricated and tested for corrosion resisting properties by immersion in boiling 20% HCl for 48 hours. The results of these tests are shown below in Table 2.

Table 2

## FORTY-EIGHT HOUR CORROSION TESTS OF VARIOUS TITANIUM-TANTALUM ALLOYS IN BOILING 20% HCl

| Heat No. | Composition              | Corrosion Rate, Mils/Year |
|----------|--------------------------|---------------------------|
| T-980    | Ti-50Ta-5Cr              | 3.6                       |
| T-981    | Ti-52Ta-5Cr              | 6.4                       |
| T-982    | Ti-54Ta-5Cr              | 3.9                       |
| T-983    | Ti-50Ta-5Cr              | 6.2                       |
| T-984    | Ti-58Ta-5Cr              | 6.2                       |
| T-985    | Ti-60Ta-5Cr              | 5.2                       |
| T-986    | Ti-50Ta-3.5Cr-1.5Fe      | 8.4                       |
| T-987    | Ti-52Ta-3.5Cr-1.5Fe      | 7.2                       |
| T-988    | Ti-54Ta-3.5Cr-1.5Fe      | 8.8                       |
| T-989    | Ti-56Ta-3.5Cr-1.5Fe      | 6.6                       |
| T-990    | Ti-58Ta-3.5Cr-1.5Fe      | 3.5                       |
| T-991    | Ti-60Ta-3.5Cr-1.5Fe      | 3.2                       |
| T-992    | Ti-50Ta-8.5V-1.5Al       | 4.0                       |
| T-993    | Ti-52Ta-8.5V-1.5Al       | 1.4                       |
| T-994    | Ti-54Ta-8.5V-1.5Al       | 1.3                       |
| T-995    | Ti-56Ta-8.5V-1.5Al       | 2.6                       |
| T-996    | Ti-58Ta-8.5V-1.5Al       | 1.7                       |
| T-997    | Ti-60Ta-8.5V-1.5Al       | 2.0                       |
| T-1001   | Ti-40Ta-10Cb-5Cr         | 2.7                       |
| T-1002   | Ti-50Ta-10Cb-5Cr         | 7.9                       |
| T-1003   | Ti-40Ta-10Cb-3.5Cr-1.5Fe | 10.5                      |
| T-1004   | Ti-50Ta-10Cb-3.5Cr-1.5Fe | 12.0                      |
| T-1005   | Ti-40Ta-10Cb-8.5V-1.5Al  | 4.2                       |
| T-1006   | Ti-50Ta-10Cb-8.5V-1.5Al  | 7.3                       |
| T-1007   | Ti-55Ta-5Cr-0.2O         | 4.5                       |
| T-1008   | Ti-55Ta-5Cr-0.3O         | 4.7                       |
| T-1009   | Ti-55Ta-3.5Cr-1.5Fe-0.2O | 2.1                       |
| T-1010   | Ti-55Ta-3.5Cr-1.5Fe-0.3O | 3.4                       |
| T-1011   | Ti-55Ta-8.5V-1.5Al-0.2O  | 1.5                       |
| T-1012   | Ti-55Ta-8.5V-1.5Al-0.3O  | 1.9                       |
| T-285    | Ti-40Ta-10Cb-5Cr         | 7.8                       |
| 9562     | Ti-50Ta-10V              | 8.2                       |
| 9563     | Ti-60Ta-10V              | 0.6                       |
| 9564     | Ti-55Ta-5V               | 0.3                       |

1 N.D. - No determination.

2 Surface flaw in specimen.

It will be seen from Tables 1 and 2 above that alloys of this invention show excellent corrosion resistant properties. Materials resisting corrosion to the extent that their corrosion rates are less than 50 mils per year in any given medium are rated as Class B, while those showing less than 5 mils per year are rated as Class A. It is evident by comparison with alloys of 50% titanium, and 50% tantalum, or 50% titanium, 40% tantalum, and 10% columbium, that the corrosion resistance of these alloys has not been materially affected by the addition of beta stabilizers according to this invention, and within the limits hereinbefore defined.

To determine thermal stability, the same types of alloys tested for corrosion were fabricated to sheet in the same manner as those whose properties are shown in Tables 1 and 2 (many of these being the same heats) and annealed, exposed to elevated temperature and tested for strength and ductility. The sheets were annealed at 1400° F. or in some cases 1500° F. for 1/2 to 1 hour, air-cooled, then heated for from 6 to 24 hours at mostly from 500° F. to 800° F. Specimens were prepared and tensile strength (ultimate and yield) and elongation determined on some, while on others bend tests were run to indicate ductility. Bend tests show the minimum bend radius, expressed as times the sheet thickness, which could be made in a specimen without cracking; such a test correlates well with ductility indicated by elongation during tensile testing. In each case a specimen of the alloy as annealed was tested to provide a comparison with that which had been exposed to elevated temperature, and the results are shown in Table 3 below.

Table 3

## THERMAL STABILITY OF VARIOUS TITANIUM-TANTALUM ALLOYS

| Heat No. | Composition  | Thermal Treatment                       | Tensile Properties |            |                 | Bend Properties, Min. T |
|----------|--------------|-----------------------------------------|--------------------|------------|-----------------|-------------------------|
|          |              |                                         | UTS, K.s.i.        | YS, K.s.i. | Elong., Percent |                         |
| 9151     | Ti-50Ta      | 1,400 F., 1/2 Hr. AC                    | 88                 | 50         | 24              |                         |
| 9151     | Ti-50Ta      | 1,400 F., 1/2 Hr. AC+800 F., 24 Hrs. AC | 145                | 145        | 0               |                         |
| 9151     | Ti-50Ta      | 1,400 F., 1/2 Hr. AC                    |                    |            |                 | 1.9                     |
| 9151     | Ti-50Ta      | 1,400 F., 1/2 Hr. AC+500 F., 8 Hrs. AC  |                    |            |                 | 5.7                     |
| 9151     | Ti-50Ta      | 1,400 F., 1/2 Hr. AC+600 F., 6 Hrs. AC  |                    |            |                 | (2)                     |
| 9151     | Ti-50Ta      | 1,400 F., 1/2 Hr. AC+800 F., 24 Hrs. AC |                    |            |                 | (2)                     |
| 9187     | Ti-40Ta-10Cb | 1,400 F., 1/2 Hr. AC                    | 100                | 44         | 28              |                         |
| 9187     | Ti-40Ta-10Cb | 1,400 F., 1/2 Hr. AC+400 F., 6 Hrs. AC  | 100                | 94         | 18              |                         |
| 9187     | Ti-40Ta-10Cb | 1,400 F., 1/2 Hr. AC+500 F., 6 Hrs. AC  | 116                | 116        | 10              |                         |
| 9187     | Ti-40Ta-10Cb | 1,400 F., 1/2 Hr. AC+800 F., 6 Hrs. AC  | 162                | 162        | 0               |                         |
| 9187     | Ti-40Ta-10Cb | 1,400 F., 1/2 Hr. AC+800 F., 24 Hrs. AC | 143                | (1)        |                 |                         |
| 9189     | Ti-40Ta-10Cb | 1,400 F., 1/2 Hr. AC                    | 106                | 38         | 31              |                         |
| 9189     | Ti-40Ta-10Cb | 1,400 F., 1/2 Hr. AC+500 F., 6 Hrs. AC  | 125                |            | 8               |                         |
| 9189     | Ti-40Ta-10Cb | 1,400 F., 1/2 Hr. AC+600 F., 6 Hrs. AC  | 139                | (1)        |                 |                         |
| T-284    | Ti-70Ta      | 1,400 F., 1/2 Hr. AC                    | 107                | 51         | 13              |                         |
| T-284    | Ti-70Ta      | 1,400 F., 1/2 Hr. AC+600 F., 6 Hrs. AC  | 119                | 115        | 7               |                         |
| T-284    | Ti-70Ta      | 1,400 F., 1/2 Hr. AC                    |                    |            |                 | 1.3                     |
| T-284    | Ti-70Ta      | 1,400 F., 1/2 Hr. AC+600 F., 96 Hrs. AC |                    |            |                 | (2)                     |

Table 3—Continued

## THERMAL STABILITY OF VARIOUS TITANIUM-TANTALUM ALLOYS

| Heat No. | Composition             | Thermal Treatment                       | Tensile Properties |            |                 | Bend Properties, Min. T |
|----------|-------------------------|-----------------------------------------|--------------------|------------|-----------------|-------------------------|
|          |                         |                                         | UTS, K.s.i.        | YS, K.s.i. | Elong., Percent |                         |
| 9458     | Ti-40Ta-10Cb-2V         | 1,400 F., 1 Hr. AC                      | 103                | 50         | 18              |                         |
| 9458     | Ti-40Ta-10Cb-2V         | 1,400 F., 1 Hr. AC+600 F., 6 Hrs. AC    | 116                | 115        | 11              |                         |
| 9459     | Ti-40Ta-10Cb-5V         | 1,400 F., 1 Hr. AC                      | 89                 | 84         | 16              |                         |
| 9459     | Ti-40Ta-10Cb-5V         | 1,400 F., 1 Hr. AC+600 F., 6 Hrs. AC    | 97                 | 91         | 8               |                         |
| T-78     | Ti-40Ta-10Cb-7V         | 1,400 F., 1/2 Hr. AC                    | 92                 | 86         | 13              |                         |
| T-78     | Ti-40Ta-10Cb-7V         | 1,400 F., 1/2 Hr. AC+800 F., 24 Hrs. AC | 93                 | 87         | 13              |                         |
| T-79     | Ti-40Ta-10Cb-12V        | 1,400 F., 1/2 Hr. AC                    | 102                | 96         | 15              |                         |
| T-79     | Ti-40Ta-10Cb-12V        | 1,400 F., 1/2 Hr. AC+800 F., 24 Hrs. AC | 103                | 100        | 15              |                         |
| T-81     | Ti-40Ta-10Cb-20V        | 1,400 F., 1/2 Hr. AC                    | 119                | 111        | 11              |                         |
| T-81     | Ti-40Ta-10Cb-20V        | 1,400 F., 1/2 Hr. AC+800 F., 24 Hrs. AC | 125                | 118        | 17              |                         |
| 9461     | Ti-40Ta-10Cb-3Cr        | 1,400 F., 1 Hr. AC                      | 110                | 101        | 12              |                         |
| 9461     | Ti-40Ta-10Cb-3Cr        | 1,400 F., 1 Hr. AC+600 F., 6 Hrs. AC    | 111                | 109        | 9               |                         |
| 9461     | Ti-40Ta-10Cb-3Cr        | 1,400 F., 1 Hr. AC+800 F., 6 Hrs. AC    | 115                | 112        | 6               |                         |
| T-285    | Ti-40Ta-10Cb-5Cr        | 1,400 F., 1/2 Hr. AC                    | 93                 | 91         | 16              |                         |
| T-285    | Ti-40Ta-10Cb-5Cr        | 1,400 F., 1/2 Hr. AC+600 F., Hrs. AC    | 98                 | 95         | 16              |                         |
| T-285    | Ti-40Ta-10Cb-5Cr        | 1,400 F., 1/2 Hr. AC+600 F., 6 Hrs. AC  | 100                | 98         | 15              |                         |
| 9562     | Ti-50Ta-10V             | 1,500 F., 1/2 Hr. AC                    | 109                | 102        | 15              |                         |
| 9562     | Ti-50Ta-10V             | 1,500 F., 1/2 Hr. AC+800 F., 48 Hrs. AC | 111                | 106        | 7               |                         |
| T-286    | Ti-55Ta-5Cr             | 1,400 F., 1/2 Hr. AC                    | 121                | 117        | 8               |                         |
| T-286    | Ti-55Ta-5Cr             | 1,400 F., 1/2 Hr. AC+600 F., 6 Hrs. AC  | 124                | 120        | 8               |                         |
| T-122    | Ti-40Ta-20Cb            | 1,400 F., 1/2 Hr. AC                    |                    |            | 4.4             |                         |
| T-122    | Ti-40Ta-20Cb            | 1,400 F., 1/2 Hr. AC+600 F., 24 Hrs. AC |                    |            | 3.9             |                         |
| T-123    | Ti-40Ta-20V             | 1,400 F., 1/2 Hr. AC                    |                    |            | 2.4             |                         |
| T-123    | Ti-40Ta-20V             | 1,400 F., 1/2 Hr. AC+600 F., 24 Hrs. AC |                    |            | 3.1             |                         |
| T-71     | Ti-40Ta-10Cb-8.5V-1.5Al | 1,400 F., 1/2 Hr. AC                    |                    |            | 4               |                         |
| T-71     | Ti-40Ta-10Cb-8.5V-1.5Al | 1,400 F., 1/2 Hr. AC+500 F., 24 Hrs. AC |                    |            | 2.6             |                         |
| T-72     | Ti-40Ta-10Cb-10V-1.8Al  | 1,400 F., 1/2 Hr. AC                    |                    |            | 2.9             |                         |
| T-72     | Ti-40Ta-10Cb-10V-1.8Al  | 1,400 F., 1/2 Hr. AC+500 F., 24 Hrs. AC |                    |            | 2.3             |                         |
| T-73     | Ti-40Ta-10Cb-12V-2.1Al  | 1,400 F., 1/2 Hr. AC                    |                    |            | 3.2             |                         |
| T-73     | Ti-40Ta-10Cb-12V-2.1Al  | 1,400 F., 1/2 Hr. AC+500 F., 24 Hrs. AC |                    |            | 2.2             |                         |
| T-289    | Ti-35Ta-20Cb-10V-1.8Al  | 1,400 F., 1/2 Hr. AC                    | 119                | 118        | 7               |                         |
| T-289    | Ti-35Ta-20Cb-10V-1.8Al  | 1,400 F., 1/2 Hr. AC+800 F., 6 Hrs. AC  | 132                | 128        | 8               |                         |
| T-290    | Ti-35Ta-15Cb-10V-1.8Al  | 1,400 F., 1/2 Hr. AC                    | 115                | 110        | 15              |                         |
| T-290    | Ti-35Ta-15Cb-10V-1.8Al  | 1,400 F., 1/2 Hr. AC+800 F., 6 Hrs. AC  | 119                | 115        | 17              |                         |
| T-511    | Ti-60Ta-8.5V-1.5Al      | 1,500 F., 1/2 Hr. AC                    |                    |            | 1.9             |                         |
| T-511    | Ti-60Ta-8.5V-1.5Al      | 1,500 F., 1/2 Hr. AC+800 F., 6 Hrs. AC  |                    |            | 2.2             |                         |
| T-512    | Ti-65Ta-8.5V-1.5Al      | 1,500 F., 1/2 Hr. AC+800 F., 6 Hrs. AC  |                    |            | 2.0             |                         |
| T-513    | Ti-60Ta-6V-1Al          | 1,500 F., 1/2 Hr. AC                    |                    |            | 2.5             |                         |
| T-513    | Ti-60Ta-6V-1Al          | 1,500 F., 1/2 Hr. AC+800 F., 6 Hrs. AC  |                    |            |                 |                         |
| T-514    | Ti-50Ta-10Cb-6V-1Al     | 1,500 F., 1/2 Hr. AC                    |                    |            |                 |                         |
| T-514    | Ti-50Ta-10Cb-6V-1Al     | 1,500 F., 1/2 Hr. AC+800 F., 6 Hrs. AC  |                    |            | 1.4             |                         |
| T-287    | Ti-40Ta-10Cb-1Fe        | 1,400 F., 1/2 Hr. AC                    | 100                | 87         | 17              |                         |
| T-287    | Ti-40Ta-10Cb-1Fe        | 1,400 F., 1/2 Hr. AC+600 F., 6 Hrs. AC  | 134                | 134        | 1               |                         |
| T-288    | Ti-40Ta-10Cb-2Fe        | 1,400 F., 1/2 Hr. AC                    | 113                | 110        | 17              |                         |
| T-288    | Ti-40Ta-10Cb-2Fe        | 1,400 F., 1/2 Hr. AC+600 F., 6 Hrs. AC  | 119                | 117        | 16              |                         |
| T-288    | Ti-40Ta-10Cb-2Fe        | 1,400 F., 1/2 Hr. AC+800 F., 6 Hrs. AC  | 122                | 118        | 9               |                         |
| T-291    | Ti-40Ta-10Cb-4Mn        | 1,400 F., 1/2 Hr. AC                    | 116                | 111        | 16              |                         |
| T-291    | Ti-40Ta-10Cb-4Mn        | 1,400 F., 1/2 Hr. AC+600 F., 6 Hrs. AC  | 116                | 113        | 19              |                         |
| T-291    | Ti-40Ta-10Cb-4Mn        | 1,400 F., 1/2 Hr. AC+800 F., 24 Hrs. AC | 123                | 114        | 11              |                         |
| T-292    | Ti-40Ta-10Cb-6W         | 1,400 F., 1/2 Hr. AC                    |                    |            | 1.9             |                         |
| T-292    | Ti-40Ta-10Cb-6W         | 1,400 F., 1/2 Hr. AC+800 F., 6 Hrs. AC  |                    |            | 1.2             |                         |
| T-292    | Ti-40Ta-10Cb-6W         | 1,400 F., 1/2 Hr. AC+800 F., 24 Hrs. AC |                    |            | 1.9             |                         |

<sup>1</sup> Brittle, no yield.<sup>2</sup> Brittle.

The results obtained on the 50% titanium, 50% tantalum alloy, as well as the 50% titanium, 40% tantalum, 10% columbium alloys showed a marked loss in ductility when these alloys were heated as low as 400° F. for 6 hours and complete loss of ductility and glass hard brittleness after being heated to 800° F. for 24 hours. Heat T-284, which was made from an alloy containing 70% tantalum, dropped in elongation from 13% to 7% after heating for 6 hours at 600° F. In comparison, the ductilities of alloys containing beta stabilizers, within the ranges herein described, show little significant reduction in ductility after heating up to 800° F. for 24 hours. Those containing 5 to 10% beta stabilizers show excellent retention of ductility, considering, of course, the limits of possible testing error. Inclusion of up to about 2% aluminum tends to improve thermal stability, and inclusion of up to this amount of this optional alloying

element enhances the corrosion resistance somewhat as will be seen by reference to Table 2.

Further tests were run to determine the thermal stability of alloys of this invention under stress. This is a characteristic that is valuable when material is employed to fabricate structural members which may be required to operate under stress as well as at elevated temperature, as for instance autoclave parts. Specimens were annealed and then maintained under stress of from 25,000 to 70,000 p.s.i. at temperatures of 500° F. and 600° F. for 150 hours. Comparison of ductilities, shown by elongation percentages, indicated little difference between specimens of alloys of this invention only annealed and after thermal stress treatment, while an alloy of 40% Ta, 10% Cb, balance Ti (Heat 9187) showed complete loss of ductility. The results of these tests are shown in Table 4 below.

Table 4

## THERMAL STRESS STABILITY OF VARIOUS TITANIUM-TANTALUM ALLOYS

| Heat No. | Composition     | Annealing Treatment  | Exposure    |                |            | Def. Percent | Subsequent Tensile Properties |            |                  |
|----------|-----------------|----------------------|-------------|----------------|------------|--------------|-------------------------------|------------|------------------|
|          |                 |                      | Temp., ° F. | Stress, K.s.i. | Time, Hrs. |              | UTS, K.s.i.                   | YS, K.s.i. | Elong., Percent  |
| 9187     | Ti-40Ta-10Cb    | 1,400 F., 1/2 Hr. AC | 500         |                | 25         | 150          | Neg.                          | 136        | ( <sup>1</sup> ) |
| 9187     | Ti-40Ta-10Cb    | 1,400 F., 1/2 Hr. AC | Room Temp.  |                | Tensile    |              | 100                           | 44         | 28               |
| 9458     | Ti-40Ta-10Cb-2V | 1,400 F., 1 Hr. AC   | 500         |                | 25         | 150          | Neg.                          | 131        | 9                |
| 9458     | Ti-40Ta-10Cb-2V | 1,400 F., 1 Hr. AC   | Room Temp.  |                | Tensile    |              | 103                           | 50         | 18               |
| 9459     | Ti-40Ta-10Cb-5V | 1,400 F., 1/2 Hr. AC | 500         |                | 25         | 150          | Neg.                          | 107        | 105              |

Table 4—Continued

| Heat No. | Composition             | Annealing Treatment            | Exposure    |                |            | Def., Percent | Subsequent Tensile Properties |            |                 |
|----------|-------------------------|--------------------------------|-------------|----------------|------------|---------------|-------------------------------|------------|-----------------|
|          |                         |                                | Temp., ° F. | Stress, K.s.i. | Time, Hrs. |               | UTS, K.s.i.                   | YS, K.s.i. | Elong., Percent |
| 9459     | Ti-40Ta-10Cb-5V         | 1,400 F., $\frac{1}{2}$ Hr. AC | 500         | 40             | 150        | Neg.          | 114                           | 112        | 22              |
| 9459     | Ti-40Ta-10Cb-7V         | 1,400 F., $\frac{1}{2}$ Hr. AC | Room Temp.  | 60             | 150        | 0.0           | 89                            | 84         | 16              |
| T-78     | Ti-40Ta-10Cb-7V         | 1,400 F., $\frac{1}{2}$ Hr. AC | 500         | —              | —          | —             | 106                           | 102        | 7               |
| T-78     | Ti-40Ta-10Cb-7V         | 1,400 F., $\frac{1}{2}$ Hr. AC | Room Temp.  | —              | —          | —             | 90                            | 84         | 18              |
| 9460     | Ti-40Ta-10Cb-10V        | 1,400 F., 1 Hr. AC             | 500         | 25             | 150        | 0.0           | 106                           | 104        | 6               |
| 9460     | Ti-40Ta-10Cb-10V        | 1,400 F., 1 Hr. AC             | Room Temp.  | —              | —          | —             | 100                           | 96         | 13              |
| T-79     | Ti-40Ta-10Cb-12V        | 1,400 F., $\frac{1}{2}$ Hr. AC | 500         | 60             | 150        | 0.0           | 105                           | 100        | 17              |
| T-79     | Ti-40Ta-10Cb-12V        | 1,400 F., $\frac{1}{2}$ Hr. AC | 600         | 60             | 150        | 0.06          | 110                           | 107        | 13              |
| T-79     | Ti-40Ta-10Cb-12V        | 1,400 F., $\frac{1}{2}$ Hr. AC | Room Temp.  | —              | —          | —             | 102                           | 96         | 15              |
| T-80     | Ti-40Ta-10Cb-16V        | 1,400 F., $\frac{1}{2}$ Hr. AC | 600         | 65             | 150        | 0.02          | 119                           | 114        | 15              |
| T-80     | Ti-40Ta-10Cb-16V        | 1,400 F., $\frac{1}{2}$ Hr. AC | Room Temp.  | —              | —          | —             | 115                           | 109        | 14              |
| T-81     | Ti-40Ta-10Cb-20V        | 1,400 F., $\frac{1}{2}$ Hr. AC | 600         | 60             | 150        | 0.0           | 120                           | 117        | 15              |
| T-81     | Ti-40Ta-10Cb-20V        | 1,400 F., $\frac{1}{2}$ Hr. AC | Room Temp.  | —              | —          | —             | 125                           | 118        | 17              |
| 9461     | Ti-40Ta-10Cb-3Cr        | 1,400 F., 1 Hr. AC             | 500         | 45             | 150        | Neg.          | 120                           | 119        | 16              |
| 9461     | Ti-40Ta-10Cb-3Cr        | 1,400 F., 1 Hr. AC             | Room Temp.  | —              | —          | —             | 110                           | 101        | 12              |
| T-285    | Ti-40Ta-10Cb-5Cr        | 1,400 F., $\frac{1}{2}$ Hr. AC | 500         | 70             | 150        | 0.95          | 95                            | 90         | 11              |
| T-285    | Ti-40Ta-10Cb-5Cr        | 1,400 F., $\frac{1}{2}$ Hr. AC | Room Temp.  | —              | —          | —             | 96                            | 92         | 13              |
| 9562     | Ti-50Ta-10V             | 1,500 F., $\frac{1}{2}$ Hr. AC | 600         | 40             | 150        | 0.0           | 121                           | —          | 6               |
| 9562     | Ti-50Ta-10V             | 1,500 F., $\frac{1}{2}$ Hr. AC | Room Temp.  | —              | —          | —             | 106                           | 102        | 15              |
| T-286    | Ti-55Ta-5Cr             | 1,400 F., $\frac{1}{2}$ Hr. AC | 600         | 60             | 150        | 0.0           | 135                           | 127        | 10              |
| T-286    | Ti-55Ta-5Cr             | 1,400 F., $\frac{1}{2}$ Hr. AC | Room Temp.  | —              | —          | —             | 121                           | 117        | 7               |
| T-122    | Ti-40Ta-20Cb            | 1,400 F., $\frac{1}{2}$ Hr. AC | 600         | 50             | 150        | 0.0           | 110                           | 106        | 4               |
| T-122    | Ti-40Ta-20Cb            | 1,400 F., $\frac{1}{2}$ Hr. AC | Room Temp.  | —              | —          | —             | 83                            | 70         | 7               |
| T-71     | Ti-40Ta-10Cb-8.5V-1.5Al | 1,400 F., $\frac{1}{2}$ Hr. AC | 600         | 60             | 150        | 0.02          | 121                           | 115        | 16              |
| T-71     | Ti-40Ta-10Cb-8.5V-1.5Al | 1,400 F., $\frac{1}{2}$ Hr. AC | Room Temp.  | —              | —          | —             | 115                           | 109        | 15              |
| T-72     | Ti-40Ta-10Cb-10V-1.8Al  | 1,400 F., $\frac{1}{2}$ Hr. AC | 600         | 60             | 150        | 0.0           | 124                           | 119        | 11              |
| T-72     | Ti-40Ta-10Cb-10V-1.8Al  | 1,400 F., $\frac{1}{2}$ Hr. AC | Room Temp.  | —              | —          | —             | 125                           | 119        | 12              |
| T-73     | Ti-40Ta-10Cb-12V-2.1Al  | 1,400 F., $\frac{1}{2}$ Hr. AC | 600         | 60             | 150        | 0.0           | 134                           | 125        | 19              |
| T-73     | Ti-40Ta-10Cb-12V-2.1Al  | 1,400 F., $\frac{1}{2}$ Hr. AC | Room Temp.  | —              | —          | —             | 137                           | 127        | 16              |
| T-289    | Ti-35Ta-20Cb-10V-1.8Al  | 1,400 F., $\frac{1}{2}$ Hr. AC | 600         | 60             | 150        | 0.0           | 126                           | 121        | 7               |
| T-289    | Ti-35Ta-20Cb-10V-1.8Al  | 1,400 F., $\frac{1}{2}$ Hr. AC | Room Temp.  | —              | —          | —             | 119                           | 118        | 7               |
| T-290    | Ti-35Ta-15Cb-10V-1.8Al  | 1,400 F., $\frac{1}{2}$ Hr. AC | 600         | 60             | 150        | 0.05          | 121                           | 114        | 14              |
| T-290    | Ti-35Ta-15Cb-10V-1.8Al  | 1,400 F., $\frac{1}{2}$ Hr. AC | Room Temp.  | —              | —          | —             | 115                           | 110        | 15              |
| T-511    | Ti-60Ta-8.5V-1.5Al      | 1,400 F., $\frac{1}{2}$ Hr. AC | 600         | 60             | 150        | 0.0           | 141                           | 135        | 7               |
| T-511    | Ti-60Ta-8.5V-1.5Al      | 1,500 F., $\frac{1}{2}$ Hr. AC | Room Temp.  | —              | —          | —             | 133                           | 128        | 8               |
| T-512    | Ti-65Ta-8.5V-1.5Al      | 1,500 F., $\frac{1}{2}$ Hr. AC | 600         | 60             | 150        | 0.0           | 148                           | 138        | 5               |
| T-512    | Ti-65Ta-8.5V-1.5Al      | 1,500 F., $\frac{1}{2}$ Hr. AC | Room Temp.  | —              | —          | —             | 146                           | 141        | 8               |
| T-513    | Ti-60Ta-6V-1Al          | 1,500 F., $\frac{1}{2}$ Hr. AC | 600         | 60             | 150        | 0.0           | 131                           | 126        | 10              |
| T-513    | Ti-60Ta-6V-1Al          | 1,500 F., $\frac{1}{2}$ Hr. AC | Room Temp.  | —              | —          | —             | 120                           | 115        | 8               |
| T-514    | Ti-50Ta-10Cb-6V-1Al     | 1,500 F., $\frac{1}{2}$ Hr. AC | 600         | 60             | 150        | 0.03          | 125                           | 120        | 7               |
| T-514    | Ti-50Ta-10Cb-6V-1Al     | 1,500 F., $\frac{1}{2}$ Hr. AC | Room Temp.  | —              | —          | —             | 121                           | 115        | 9               |
| T-291    | Ti-40Ta-10Cb-4Mn        | 1,400 F., $\frac{1}{2}$ Hr. AC | 600         | 60             | 150        | 0.0           | 134                           | 129        | 10              |
| T-291    | Ti-40Ta-10Cb-4Mn        | 1,400 F., $\frac{1}{2}$ Hr. AC | Room Temp.  | —              | —          | —             | 115                           | 112        | 15              |

<sup>1</sup> Brittle; broke outside gage length.

A preferred alloy showing an excellent combination of corrosion resistance and thermal stability contains 50% tantalum, 8.5% vanadium, 1.5% aluminum, balance titanium. A similar alloy contains 50% tantalum, 10% columbium, 8.5% vanadium, 1.5% aluminum, balance titanium and it will be noted that in this case 10% of the tantalum content has been replaced with columbium. Representative corrosion resistance and mechanical properties of these alloys, before and after thermal exposure, are tabulated in Table 5 below.

Table 5

ALLOY—50% Ta, 8.5% V, 1.5% Al, BALANCE Ti

| Boiling                                            | 20% HCl     | 60% H <sub>2</sub> SO <sub>4</sub> | 30% H <sub>3</sub> PO <sub>4</sub> | 3% Oxalic Acid |
|----------------------------------------------------|-------------|------------------------------------|------------------------------------|----------------|
| Corrosion Resistance, Mils per Year (48 hour test) | 1.5         | 4                                  | 4                                  | 20             |
| Mechanical Properties                              | UTS, K.s.i. | YS, K.s.i.                         | Elong., Percent                    | Bend, Min. T   |
| As Annealed                                        | 120         | 115                                | 12                                 | 2              |
| After 800° F. for 24 hours                         | 130         | 125                                | 10                                 | 2.2            |

ALLOY—40% Ta, 10% Cb, 8.5% V, 1.5% Al, BALANCE Ti

| Boiling                                            | 20% HCl | 60% H <sub>2</sub> SO <sub>4</sub> | 30% H <sub>3</sub> PO <sub>4</sub> | 3% Oxalic Acid |
|----------------------------------------------------|---------|------------------------------------|------------------------------------|----------------|
| Corrosion Resistance, Mils per year (48 hour test) | 7.5     | 7.5                                | 10                                 | 30             |

Table 5—Continued

|                            | Mechanical Properties | UTS, K.s.i. | YS, K.s.i. | Elong., Percent | Bend, Min. T |
|----------------------------|-----------------------|-------------|------------|-----------------|--------------|
| As Annealed                | 120                   | 110         | 15         | 3               |              |
| After 800° F. for 24 hours | 130                   | 120         | 13         | 3.5             |              |

The alloy containing columbium replacing part of the tantalum has the advantage of reduced cost when a combined tantalum-columbium master alloy can be used in its production. Its corrosion resistance is not appreciably poorer than the alloy containing tantalum and no columbium, and it may advantageously be employed under conditions in which it may be exposed to less corrosive media than those used for test results.

The amounts of the various alloying constituents in the compositions of this invention are critical to obtain the benefits and desirable properties imparted thereby. The tantalum content in combination with the titanium appears to be in large measure responsible for the corrosion resistant properties of the alloys. Adequate corrosion resistance will not be obtained if the tantalum content is less than 40%, or, if part of the tantalum is replaced by columbium, the tantalum content should be at least 35%. If more than 70% tantalum is employed, a large part of the extremely desirable low cost advantage of the alloys of this invention will be lost. It is extremely significant that the alloys of this invention provide corrosion resistant properties approaching those of pure tantalum, yet contain 70% or less of tantalum, which is very expensive material. If percentages of tantalum higher than 70% are employed, the corrosion resistant properties may correspond closely to those of pure tantalum but at the same time, due to increased alloying and processing

costs, the more complex compositions may show little, if any, significant cost advantage.

The percentages of beta stabilizing elements are critical to obtain the desirable stability characteristics without affecting to an appreciable degree the excellent corrosion resistant properties of the alloys. Less than 2% beta stabilizer will not provide sufficient increase in thermal stability to be appreciable or of practical importance, and more than 20% beta stabilizer will adversely affect the corrosion resistance and in addition, some of the mechanical properties. A small amount of aluminum within the limit stated will improve the corrosion resistance, although the reason for this effect is not precisely known. In addition, the small amount of aluminum contributes to providing thermal stability in the alloy since it will to some extent reduce the tendency for precipitation of the omega phase which has a marked hardening effect on the beta matrix. More than 2.5% of aluminum will tend to more strongly stabilize the alpha phase and reduce the beneficial effects of inclusion of beta stabilizers as hereinbefore described.

The alloy of this invention may be produced by any convenient method in which the constituents are rendered molten to provide an ingot of homogenous alloy composition. Arc melting procedures may be employed, and the titanium, tantalum and other alloying constituents may be pressed into compacts and these compacts assembled into an electrode which can be melted into a cold mold crucible by the well-known consumable electrode arc melting process. It should be pointed out, however, that a homogenous ingot is necessary to obtain uniform properties, and the proper and desired effect produced by the various alloy constituents. It will be appreciated that titanium and tantalum have substantially different melting points and more than normal difficulty may be encountered in producing an ingot which is free from unmelted inclusions of the higher melting point tantalum metal. Use of tantalum in relatively finely divided powdered form, so as to obtain an initial relatively good dispersion of this material, will be helpful in producing homogeneous materials; and in addition, remelting of the ingot preferably several times will be found also effective to produce acceptable homogeneity.

The alloys of this invention possess outstanding corrosion resistant properties as will be evident from the data presented herein. At the same time the thermal stability, as indicated by retention of ductility after exposure to temperatures up to 800° F., will be satisfactory for applications involving exposure of products fabricated from these alloys at such elevated temperatures for a reasonable period of time, and also indicates a substantial immunity from thermal instability at temperatures of the order of those normally encountered in boiling aqueous solutions for an extremely long life period. It will be appreciated by those skilled in the art that an alloy of this invention can be used for long periods of time without fear of embrittlement under corrosive conditions at elevated temperatures, as for example, when employed as structural or lining materials in autoclaves, and similar relatively high temperature and pressure equipment, as well as being useful at temperatures encountered in contact with aqueous solutions even up to their boiling point more or less indefinitely.

The alloys of this invention are characterized, in addition, by substantially higher tensile strength than shown by pure tantalum or by the previously known alloys of

tantalum and titanium. Inclusion of a beta stabilizing element markedly increases the yield strength and tensile strength of the alloy. This makes it possible for thinner and lighter structural or lining members to be employed while retaining similar strength and corrosion resistant properties. It will also be found that the alloys of this invention are considerably lighter than the pure tantalum which they are capable of replacing in many applications; and this is responsible for production of a greater volume of fabricated material per pound; thus further reducing the cost of the alloy in useful form. It will be evident that a pound of an alloy according to this invention will provide substantially more sheet of a given thickness than can be obtained from a pound of pure tantalum. The alloy of this invention will be substantially stronger while at the same time possessing improved thermal stability, and corrosion resistant properties will approach those of pure tantalum.

Alloys of this invention will be found useful for many applications where corrosion resisting characteristics approaching those of pure tantalum are required. It provides such characteristics at substantially less cost than pure tantalum due to the inclusion of large proportions of other, less costly, elements.

We claim:

1. An alloy formed by melting its constituents characterized by resistance to corrosion by HCl indicated by a corrosion rate of less than 10 mils per year in boiling 20% HCl, 48 hour test, and by thermal stability indicated by substantial retention of ductility after exposure to temperatures up to about 800° F. consisting essentially of:
  - (a) about 40% by weight tantalum,
  - (b) about 10% by weight columbium,
  - (c) about 1.5% by weight aluminum, and
  - (d) about 8.5% by weight vanadium,
  - (e) balance titanium.
2. An alloy formed by melting its constituents characterized by resistance to corrosion by HCl indicated by a corrosion rate of less than 10 mils per year in boiling 20% HCl, 48 hour test, and by thermal stability indicated by substantial retention of ductility after exposure to temperatures up to about 800° F. consisting essentially of:
  - (a) about 50% by weight tantalum,
  - (b) about 1.5% by weight aluminum, and
  - (c) about 8.5% by weight vanadium,
  - (d) balance titanium.

#### References Cited in the file of this patent

#### UNITED STATES PATENTS

|    |           |                     |               |
|----|-----------|---------------------|---------------|
| 50 | 2,880,088 | Jaffee et al. ----- | Mar. 31, 1959 |
|    | 2,880,089 | Vordahl -----       | Mar. 31, 1959 |
|    | 2,882,146 | Rhodin -----        | Apr. 14, 1959 |
|    | 2,940,845 | Jaffee et al. ----- | June 14, 1960 |
| 55 | 2,948,607 | Wagener -----       | Aug. 9, 1960  |

#### FOREIGN PATENTS

|         |               |               |
|---------|---------------|---------------|
| 201,297 | Austria ----- | Dec. 27, 1958 |
|---------|---------------|---------------|

#### OTHER REFERENCES

Reactive Metals V, 2 reprinted from Metallurgical Society Conferences, Proceedings of the Third Annual Conference sponsored by Niagara Frontier Section in cooperation with The Metallurgical Society, Aime, Buffalo, New York, May 27-29, 1958, Interscience Publishers (pages 497-499 relied upon).